

Feb. 6, 1962

C. W. VIGOR

3,020,152

EXHAUST VALVE STEEL

Filed May 2, 1960



0.63-0.68% CARBON  
8.75-10.25% MANGANESE  
20.5-22.5% CHROMIUM  
2.2 -2.8% MOLYBDENUM  
0.34-0.38% NITROGEN  
0.02-0.03% BORON  
0-0.5% SILICON  
BALANCE - IRON

INVENTOR.  
*Charles W. Vigor*  
BY  
*B. N. Shamp*  
ATTORNEY

## 1

3,020,152

## EXHAUST VALVE STEEL

Charles W. Vigor, East Detroit, Mich., assignor to General Motors Corporation, Detroit, Mich., a corporation of Delaware

Filed May 2, 1960, Ser. No. 26,293

7 Claims. (Cl. 75—126)

This invention relates to an austenitic stainless steel having outstanding high-temperature properties and particularly to an internal combustion engine exhaust valve formed of such a steel.

During the past few years numerous stainless steels, including austenitic stainless steels, have been developed and used commercially for high-temperature applications. Exhaust valves for internal combustion engines, for example, have been formed of austenitic stainless steels containing high alloy contents. However, none of these steels has been completely satisfactory in all respects as an exhaust valve material. While some of the alloy steels commercially available today have a desirable low nickel content and low alloy content generally, these steels do not possess the hardness necessary to avoid excessive tip wear in single-piece valves. Other valve steels have inadequate high-temperature strength or poor workability.

Accordingly, it is a principal object of the present invention to provide an austenitic stainless steel which completely satisfies today's stringent physical property requirements for exhaust valves of gasoline engines but which has a relatively low strategic alloy content. The austenitic stainless steel hereinafter described possesses the desirable combination of excellent high-temperature strength, oxidation resistance and room-temperature hardness while retaining a satisfactory degree of forgeability.

Other objects and advantages of this invention will more fully appear from the following detailed description of a preferred embodiment, reference being made to the accompanying drawing which shows a poppet valve for an automobile engine.

The exceptionally high stress-rupture strength of the austenitic stainless steel described herein results from a balanced composition in which the percentage ranges of the various elements present are specific and relatively narrow. This stainless steel consists essentially of about 0.63% to 0.68% total carbon, silicon not in excess of 0.5%, 8.75% to 10.25% manganese, 20.5% to 22.5% chromium, 2.2% to 2.8% molybdenum, 0.34% to 0.38% nitrogen, 0.02% to 0.03% boron and the balance iron. Outstanding results have been obtained with alloy steel exhaust valves having a nominal chemical composition of approximately 0.65% carbon, 0.25% silicon, 9.5% manganese, 21.5% chromium, 2.5% molybdenum, 0.36% nitrogen, 0.025% boron and the balance iron. It will be noted that, unlike most of the austenitic stainless steels heretofore used commercially in exhaust valves of automobile engines, the alloy described herein need not contain nickel, a relatively expensive strategic metal. The manganese and nitrogen in the aforementioned amounts promote austenite stability even in the absence of nickel.

The specific combination of constituents in the limited ranges set forth above provides the austenitic stainless steel alloy, after relatively simple heat treatment, with exceptional room-temperature hardness as well as excellent high-temperature strength. A Rockwell "C" hard-

## 2

ness of at least 38 results from solution treatment plus aging. The various elements in the alloy steel are balanced so as to maintain a high level of strength during long periods of exposure at elevated temperatures.

Carbon is present in the specific range set forth above to perform two functions. Carbon is necessary to provide a stable austenitic phase, and it also contributes to the strength and hardness of the steel at both room and elevated temperatures by forming carbides with other constituents in the alloy. As indicated above, the best combination of these effects is obtained if the aforementioned carbon range is rigidly adhered to. If the carbon content is reduced below approximately 0.63%, the room-temperature hardness of the steel is decreased. An excessively high carbon content reduces its high-temperature stress-rupture strength.

When the amount of silicon present does not exceed about 0.5%, it does not appreciably affect the strength or stability of the alloy. In general, a higher silicon content improves the oxidation resistance of stainless steel alloys. However, in the case of exhaust valve steels, it has been found that a high silicon content actually is detrimental to oxidation resistance since it is incompatible with lead oxide engine deposits.

Manganese is added to the stainless steel principally for its beneficial effect in promoting a stable austenitic structure. It has been found advantageous to include only that amount of manganese which, in combination with the other austenite stabilizing elements (carbon and nitrogen), results in maximum long-term stability. If the quantity of manganese present in the alloy is less than approximately 8.75%, the high-temperature strength and oxidation resistance are reduced.

The oxidation resistance of the stainless steel is further increased to an appreciable extent by the presence of chromium. In the case of exhaust valves, the chromium content should be at least 20.5% to provide the desired oxidation resistance. The maximum amount of chromium which may be present is determined by the advisability of maintaining the proper austenite-ferrite balance since chromium has a pronounced effect in promoting ferrite formation. The chromium level is one of the major factors in determining the amount of austenite stabilizing elements (carbon, manganese and nitrogen) required to stabilize an austenitic structure. If the chromium content of the steel is increased without properly adjusting the amounts of the other elements, it produces a structure which is unstable during long periods of exposure at elevated temperatures. The resultant instability, which is manifested by a transformation into a gradually increasing amount of ferrite, reduces the high-temperature strength of the alloy steel.

Chromium also enters into reactions with carbon and iron to form complex carbides which increase the strength and hardness of the stainless steel at both room and elevated temperatures. It should be noted that chromium restricts the formation of austenite under high-temperature equilibrium conditions. However, it anomalously also promotes the retention of austenite at low temperatures because of the sluggishness it imparts to the kinetics of the austenite-ferrite phase transformation.

The molybdenum contributes principally to the high-temperature strength of the steel through solution hardening of the austenitic matrix. Since molybdenum also tends to promote the formation of ferrite, the carbon, man-

ganese and nitrogen contents should be adjusted accordingly.

The stainless steel alloy described herein contains nitrogen in the amount specified because of the austenite-stabilizing influence of this element. If nitrogen is omitted, the carbon and manganese in the steel are ineffective to maintain the alloy as a stable austenitic material. As in the case of manganese, it has been found desirable to keep the nitrogen content at the lowest level commensurate with the requirement for phase stability. A nitrogen content in excess of approximately 0.38% lowers the high-temperature strength of the steel and results in undesirable carbide precipitation reactions. These reactions produce a lamellar type of carbide precipitate rather than a uniform dispersion of carbide. It appears that the nitrogen is not in the precipitate but remains in the parent austenite phase.

Boron is included in the present stainless steel alloy to improve the long-time high-temperature strength and ductility. It is believed that boron preferentially locates in the grain boundary areas of the alloy and prevents the precipitation of carbides in these areas. Consequently, it is possible for the resultant stainless steel to sustain creep type of deformation for a longer period of time without initiating ruptures at grain boundaries. Such ruptures normally indicate the beginning of high-temperature stress-rupture type of failure. A boron content less than about 0.02% does not provide the desired high-temperature strength and ductility, while the addition of boron in an amount greater than approximately 0.03% is detrimental to forgeability and oxidation resistance. The resultant decrease in forgeability causes hot shortness, while the reduction in oxidation resistance is evidenced by a nonadherent oxide which forms at high temperatures.

The initial level of strength in this alloy is dependent upon controlled precipitation of complex carbides from a solid solution matrix. This is accomplished by heat treatment, the strength being determined by the type and amount of the precipitate in relation to the nature of the matrix. Maintaining a high level of strength at elevated temperatures over a long period of time requires that precipitation reactions and matrix structure composition remain in an optimum balance. Since it is obviously impossible to readjust the chemical composition of an exhaust valve while in service, the optimum balance for long-term properties must be provided by the original chemical composition, of course. As indicated above, this goal has been achieved in the present austenitic steel alloy to an outstanding degree.

The principal problem in achieving the aforementioned balance involves maintaining the proper amounts of those elements which promote the formation and stabilization of an austenitic structure in relation to those which favor the formation of ferrite. In the above-described stainless steel the carbon, manganese and nitrogen tend to produce a stable austenitic structure, while the chromium and molybdenum favor the formation of ferrite. This delicate balance is further complicated by the requirement for precipitation hardening because some of these same elements affecting the austenite-ferrite balance also react to form the precipitating compounds. These compounds consist principally of complex carbides of iron and chromium. Since precipitation reactions are not limited to the initial heat treatment of a valve, but continue during its entire service life due to the high operating temperatures in the combustion chamber of a gasoline engine, the proper determination of a critical composition balance must be based on a time-dependent, high-temperature strength function, such as stress-to-rupture strength.

The importance of the aforementioned mechanism is indicated by the fact that the austenitic stainless steel described herein possesses outstanding high-temperature stress-rupture strength despite its relatively low strategic metal content. For example, at a temperature of 1300° F., this steel will withstand a stress of approximately 37,000 p.s.i. to 44,000 p.s.i. for 100 hours without ruptur-

ing. At 1400° F., the stress for the same rupture life is still normally in the range between 26,000 p.s.i. and 27,500 p.s.i. Even when the stainless steel is heated to a temperature of 1500° F., the stress for a 100-hour rupture life is about 15,500 p.s.i. to 17,000 p.s.i. This maximum stress for 100 hours remains in the 9,200 p.s.i. to 10,300 p.s.i. range when the temperature is increased to 1600° F. It should be noted that these excellent stress-rupture properties are obtained without sacrificing the forgeability and hardness required for exhaust valves of gasoline engines. The method of preparing the alloy steel is entirely conventional.

This austenitic stainless steel can be used in a wide variety of commercial applications because of its good workability. It can be forged or extruded without difficulty. Furthermore, the aforementioned high room-temperature hardness of the steel permits single-piece valves, which are very resistant to tip wear, to be formed of it. As indicated above, this steel also exhibits high-temperature strength considerably above that obtained with other valve steel alloys having comparable and even greater total alloy contents.

While my invention has been described by means of certain specific examples, it is to be understood that its scope is not to be limited thereby except as defined by the following claims.

I claim:

1. A poppet valve for an internal combustion engine, said valve being formed of a substantially nickel-free, austenitic stainless steel consisting essentially of about 0.63% to 0.68% carbon, 8.75% to 10.25% manganese, 20.5% to 22.5% chromium, 2.2% to 2.8% molybdenum, 0.34% to 0.38% nitrogen, 0.02% to 0.03% boron and the balance substantially all iron.
2. A heat-treated exhaust valve for a gasoline engine, said valve having a Rockwell "C" hardness of at least 38 and being formed of an austenitic stainless steel consisting essentially of about 0.63% to 0.68% carbon, 0% to 5% silicon, 8.75% to 10.25% manganese, 20.5% to 22.5% chromium, 2.2% to 2.8% molybdenum, 0.34% to 0.38% nitrogen, 0.02% to 0.03% boron and the balance substantially all iron, said valve having a stress-rupture strength of at least 26,000 p.s.i. for 100 hours at a temperature of 1400° F.
3. A one-piece, solution-treated and aged exhaust valve for a gasoline engine, said valve having a Rockwell "C" hardness at room temperature of at least 38 and being formed of an austenitic stainless steel consisting essentially of about 0.65% carbon, 0.25% silicon, 9.5% manganese, 21.5% chromium, 2.5% molybdenum, 0.36% nitrogen, 0.02% boron, and the balance substantially all iron, said valve having a stress-rupture strength of at least 26,000 p.s.i. for 100 hours at a temperature of 1400° F.
4. An austenitic stainless steel characterized by outstanding high-temperature strength, oxidation resistance and room-temperature hardness, said stainless steel consisting essentially of about 0.63% to 0.68% carbon, 8.75% to 10.25% manganese, 20.5% to 22.5% chromium, 2.2% to 2.8% molybdenum, 0.34% to 0.38% nitrogen, 0.02% to 0.03% boron and the balance substantially all iron.
5. A forgeable, nickel-free, austenitic stainless steel characterized by outstanding high-temperature strength, oxidation resistance and room-temperature hardness, said stainless steel consisting essentially of about 0.63% to 0.68% carbon, silicon not in excess of 0.5%, 8.75% to 10.25% manganese, 20.5% to 22.5% chromium, 2.2% to 2.8% molybdenum, 0.34% to 0.38% nitrogen, 0.02% to 0.03% boron and the balance substantially all iron.
6. A heat-treated, forgeable, austenitic stainless steel characterized by outstanding oxidation resistance, room temperature hardness and a stress-rupture life of at least 100 hours under a stress of 26,000 p.s.i. at a temperature of 1400° F., said stainless steel consisting essentially of about 0.63% to 0.68% carbon, 0.1% to 0.5% silicon, 8.75% to 10.25% manganese, 20.5% to 22.5% chromium, 2.2% to 2.8% molybdenum, 0.34% to 0.38% nitrogen,

0.02% to 0.03% boron and the balance substantially all iron.

7. A solution-treated and aged austenitic stainless steel having a Rockwell "C" hardness at room temperature of at least 38 and consisting essentially of about 0.63% to 0.68% carbon, 0% to 5% silicon, 8.75% to 10.25% manganese, 20.5% to 22.5% chromium, 2.2% to 2.8% molybdenum, 0.34% to 0.38% nitrogen, 0.02% to 0.03% boron and the balance substantially all iron, said steel

having a stress-rupture life of at least 100 hours under a stress of 26,000 p.s.i. at a temperature of 1400° F.

References Cited in the file of this patent

UNITED STATES PATENTS

- |           |                         |                |
|-----------|-------------------------|----------------|
| 2,764,481 | Dyrkacz et al. -----    | Sept. 25, 1956 |
| 2,814,563 | Dyrkacz et al. -----    | Nov. 26, 1957  |
| 2,948,604 | MacFarlans et al. ----- | Aug. 9, 1960   |